



US008137753B2

(12) **United States Patent**  
**Tarao et al.**

(10) **Patent No.:** **US 8,137,753 B2**  
(45) **Date of Patent:** **Mar. 20, 2012**

(54) **PAINTED GOLF BALL AND METHOD FOR PRODUCING THE SAME**

(75) Inventors: **Toshiyuki Tarao**, Kobe (JP); **Manabu Tomosada**, Kobe (JP); **Kazuhiro Tanaka**, Kobe (JP); **Kuniyasu Horiuchi**, Kobe (JP); **Takashi Sasaki**, Kobe (JP); **Hirokazu Okamoto**, Amagasaki (JP); **Masahiko Shiraishi**, Amagasaki (JP)

(73) Assignee: **SRI Sports Limited**, Kobe-Shi (JP)

(\*) Notice: Subject to any disclaimer, the term of this patent is extended or adjusted under 35 U.S.C. 154(b) by 304 days.

(21) Appl. No.: **12/631,160**

(22) Filed: **Dec. 4, 2009**

(65) **Prior Publication Data**

US 2010/0144468 A1 Jun. 10, 2010

(30) **Foreign Application Priority Data**

|               |      |       |             |
|---------------|------|-------|-------------|
| Dec. 5, 2008  | (JP) | ..... | 2008-311112 |
| Dec. 17, 2008 | (JP) | ..... | 2008-321314 |
| Nov. 10, 2009 | (JP) | ..... | 2009-257428 |

(51) **Int. Cl.**

*A63B 37/14* (2006.01)  
*A63B 37/00* (2006.01)  
*C09D 175/00* (2006.01)

(52) **U.S. Cl.** **427/316; 427/393.5; 427/412.1; 473/351; 524/501; 524/507; 525/127**

(58) **Field of Classification Search** ..... None  
See application file for complete search history.

(56) **References Cited**

U.S. PATENT DOCUMENTS

6,210,295 B1 4/2001 Yoneyama  
6,509,410 B2 1/2003 Ohira et al.  
7,141,628 B2 11/2006 Isogawa et al.

2001/0034398 A1 10/2001 Ohira et al.  
2004/0116623 A1 6/2004 Isogawa et al.  
2005/0282661 A1 12/2005 Fujisawa et al.  
2006/0178471 A1 8/2006 Sasaki et al.  
2007/0117654 A1 5/2007 Sasaki  
2010/0167847 A1\* 7/2010 Tarao et al. .... 473/378  
2011/0105247 A1\* 5/2011 Tarao et al. .... 473/378

FOREIGN PATENT DOCUMENTS

|    |               |         |
|----|---------------|---------|
| JP | 10-151224 A   | 6/1998  |
| JP | 2000-262649 A | 9/2000  |
| JP | 2001-271027 A | 10/2001 |
| JP | 2002-284836 A | 10/2002 |
| JP | 2004-187829 A | 7/2004  |
| JP | 2006-557 A    | 1/2006  |
| JP | 2006-218046 A | 8/2006  |
| JP | 2007-143660 A | 6/2007  |
| JP | 2007-260356 A | 10/2007 |

OTHER PUBLICATIONS

English translation of Japanese Office Action dated Jan. 4, 2011, for corresponding Application No. 2008-311112.

English Translation of Notice of Reasons for Allowance for corresponding Japanese Application No. 2008-311112 dated Sep. 6, 2011.

\* cited by examiner

*Primary Examiner* — David Buttner

(74) *Attorney, Agent, or Firm* — Birch, Stewart, Kolasch & Birch, LLP

(57) **ABSTRACT**

An object of the present invention is to provide a painted golf ball which is excellent in the gloss and the evenness of the paint thickness as well as the adhesion of the paint film to the golf ball body. The method for producing the golf ball of the present invention comprises applying a two-component curing type urethane-based aqueous paint including an aqueous polyol composition (A) and an aqueous polyisocyanate (B) to a golf ball body in a specific method, wherein (A) the aqueous polyol composition contains (a-1) an aqueous acrylic polyol, (a-2) an aqueous urethane polyol and (a-3) an aqueous urethane resin.

**19 Claims, 2 Drawing Sheets**



Fig.1

2

Fig.2

**PAINTED GOLF BALL AND METHOD FOR PRODUCING THE SAME**

**FIELD OF THE INVENTION**

The present invention relates to a painted golf ball and a method for producing the same.

**DESCRIPTION OF THE RELATED ART**

A conventional golf ball has a paint film on the surface of the golf ball body. The paint film is formed to protect the golf ball body from deteriorating due to the exposure of the golf ball body to a sunlight and/or the weather and to improve the appearance thereof by imparting a gloss to the golf ball body. Various paints for forming such a paint film have been developed. For example, Japanese Patent Publication No. 2001-271027 A discloses an aqueous paint composition for a golf ball, which includes a hydrophilic group-containing polyisocyanate, and a water-soluble urethane polyol having a hydroxyl value of 100 to 300 which is obtained through reaction between a polyol component and a polyisocyanate component. Japanese Patent Publication No. 2004-187829 A discloses a paint for a golf ball, which includes a polyisocyanate, and an aqueous liquid of an aqueous polyol which has a hydroxyl value from 50 mg KOH/g and below 100 mg KOH/g, and has a weight average molecular weight ranging from 4,000 to 20,000.

A golf ball is repeatedly hit and used. Therefore, the paint film for a golf ball needs to have an adhesion property against the impact. In particular, when a golf ball is hit, the golf ball body deforms. Unless the paint film covering the golf ball body does not follow the deformation of the golf ball body, the paint film tends to peel off. Further, the paint film may peel off when the golf ball is subject to the friction against the club surface when hitting the golf ball or against the ground surfaces such as sand in a bunker or rough when landing on the ground.

As a method for enhancing the adhesion of a paint film to the surface of a golf ball body, Japanese Patent Publication No. 2006-557 A discloses, for example, a method for producing a golf ball in which a marking is placed on the surface of a golf ball body, and a two-component curing type aqueous paint which includes a base material, a curing agent, and a solvent is used as an aqueous paint for forming a paint film, and a resin component for forming the marking is cured by using the curing agent included in the aqueous paint.

As a golf ball having an enhanced adhesion of a paint film to the surface of a golf ball body, Japanese Patent Publication No. 2006-218046 A discloses a golf ball, having a golf ball body and a paint film covering the golf ball body, in which the paint film is obtained by curing a paint composition which contains a carboxyl group-containing aqueous polyol, an aqueous polyisocyanate, and an aqueous polycarbodiimide.

**SUMMARY OF THE INVENTION**

In the aqueous paint disclosed in Japanese Patent Publications No. 2006-557 A and No. 2006-218046 A, although the adhesion of the paint film to the golf ball body has been improved, the leveling of the paint film was insufficient and there remains a room for further improvement from the aspect of the gloss.

Further, the two-component curing type urethane-based aqueous paint contains water as a main component of its solvent, and the solvent is not readily volatilized during a painting process. Accordingly, if the paint is applied to the

surface of the golf ball body, since the paint contains a large amount of solvent, the paint is likely to sag. Consequently, when the two-component curing type urethane-based aqueous paint is applied to the surface of a golf ball body, it is difficult to form a paint film having an even film thickness, due to the particular shape of the dimples formed on the surface of the golf ball body.

The present invention has been made in view of the above circumstances, and an object of the present invention is to provide a method for producing a painted golf ball which is excellent in the gloss and the evenness of the paint film thickness as well as the adhesion of the paint film to the golf ball body.

In one aspect of the present invention, the present invention provides a method for producing the golf ball, which comprises

applying a two-component curing type urethane-based aqueous paint containing (A) an aqueous polyol composition and (B) an aqueous polyisocyanate to a golf ball body having a surface temperature ranging from 30°C. to 80°C., wherein,

(A) the aqueous polyol composition contains (a-1) an aqueous acrylic polyol, (a-2) an aqueous urethane polyol and (a-3) an aqueous urethane resin;

a content of (a-3) the aqueous urethane resin in (A) the aqueous polyol composition ranges from 20 mass % to 80 mass %; and

a molar ratio (NCO/OH) of an isocyanate group of (B) the aqueous polyisocyanate to a hydroxyl group of (A) the aqueous polyol composition ranges from 1.25 to 2.50.

According to one aspect of the present invention, the sagging of the paint applied to the surface of the golf ball body is suppressed by controlling the surface temperature of the golf ball body within a predetermined range. Further, the two-component curing type urethane-based aqueous paint which contains (a-1) an aqueous acrylic polyol improving the gloss of the paint film, (a-2) an aqueous urethane polyol improving the adhesion of the paint film to the golf ball body, and (a-3) an aqueous urethane resin improving the tensile property of the paint film and allowing the paint film to follow the deformation of the golf ball body when hit in a predetermined content is used. The present invention configured above provides the golf ball which is excellent in the gloss of the paint film, the even thickness of the paint film, and the adhesion of the paint film to the golf ball body.

In another aspect of the present invention, the present invention provides a method for producing a golf ball, which comprises

overpainting a two-component curing type urethane-based aqueous paint containing (A) an aqueous polyol composition and (B) an aqueous polyisocyanate to a golf ball body multiple times until a paint film has a desired thickness, such that an applied amount (dry mass) of the paint per one time ranges from 5 mg to 80 mg, wherein,

(A) the aqueous polyol composition contains (a-1) an aqueous acrylic polyol, (a-2) an aqueous urethane polyol and (a-3) an aqueous urethane resin;

a content of (a-3) the aqueous urethane resin in (A) the aqueous polyol composition ranges from 20 mass % to 80 mass %;

a molar ratio (NCO/OH) of an isocyanate group of (B) the aqueous polyisocyanate to a hydroxyl group of (A) the aqueous polyol composition ranges from 1.25 to 2.50; and

a non-volatile content of the two-component curing type urethane-based aqueous paint ranges from 15 mass % to 60 mass %.

According to another aspect of the present invention, the sagging of the paint applied to the surface of the golf ball body

is suppressed by controlling the applied amount (dry mass) of the paint per one time and overpainting the paint multiple times until the paint film has a desired thickness. Further, the two-component curing type urethane-based aqueous paint which containing (a-1) an aqueous acrylic polyol improving the gloss of the paint film, (a-2) an aqueous urethane polyol improving the adhesion of the paint film to the golf ball body, and (a-3) an aqueous urethane resin improving the tensile property of the paint film and allowing the paint film to follow the deformation of the golf ball body when hit in a predetermined content is used. The present invention configured above provides the golf ball which is excellent in the gloss of the paint film, the even thickness of the paint film, and the adhesion of the paint film to the golf ball body.

In yet another aspect of the present invention, the present invention provides a golf ball produced by the method for producing the golf ball of the present invention.

According to the present invention, it is possible to obtain the golf ball which is excellent in the gloss of the paint film, the even thickness of the paint film, and the adhesion of the paint film to the golf ball body.

#### BRIEF DESCRIPTION OF THE DRAWINGS

FIG. 1 is a schematic view illustrating an embodiment applying the paint with an air gun; and

FIG. 2 is an expanded sectional view of the dimples formed on the surface of the golf ball body.

#### DESCRIPTION OF THE PREFERRED EMBODIMENT

The present invention provides a method for producing a golf ball which comprises

applying a two-component curing type urethane-based aqueous paint including an aqueous polyol composition (A) and an aqueous polyisocyanate (B) to a golf ball body having a surface temperature ranging from 30°C. to 80°C., wherein,

the aqueous polyol composition (A) contains (a-1) an aqueous acrylic polyol, (a-2) an aqueous urethane polyol and (a-3) an aqueous urethane resin;

a content of (a-3) the aqueous urethane resin in (A) the aqueous polyol composition ranges from 20 mass % to 80 mass %; and

a molar ratio (NCO/OH) of an isocyanate group of (B) the aqueous polyisocyanate to a hydroxyl group of (A) the aqueous polyol composition ranges from 1.25 to 2.50.

The present invention also provides a method for producing a golf ball which comprises

overpainting a two-component curing type urethane-based aqueous paint including an aqueous polyol composition (A) and an aqueous polyisocyanate (B) to a golf ball body multiple times until a paint film has a desired thickness, such that an applied amount (dried mass) of the paint per one time ranges from 5 mg to 80 mg, wherein,

the aqueous polyol composition (A) contains (a-1) an aqueous acrylic polyol, (a-2) an aqueous urethane polyol and (a-3) an aqueous urethane resin;

a content of (a-3) the aqueous urethane resin in (A) the aqueous polyol composition ranges from 20 mass % to 80 mass %;

a molar ratio (NCO/OH) of an isocyanate group of (B) the aqueous polyisocyanate to a hydroxyl group of (A) the aqueous polyol composition ranges from 1.25 to 2.50; and

a non-volatile content of the two-component curing type urethane-based aqueous paint ranges from 15 mass % to 60 mass %.

In the present invention, the term "aqueous" used herein includes both "water-soluble" and "water-dispersible".

#### (1) Two-Component Curing Type Urethane-Based Aqueous Paint

First, the two-component curing type urethane-based aqueous paint for a golf ball used in the present invention will be described.

The two-component curing type urethane-based aqueous paint used in the present invention forms a paint film by generating a polyurethane through curing reaction between (A) the aqueous polyol composition and (B) the aqueous polyisocyanate.

(A) The aqueous polyol composition contains (a-1) an aqueous acrylic polyol, (a-2) an aqueous urethane polyol, and (a-3) an aqueous urethane resin.

##### (1-1) Aqueous Acrylic Polyol

(a-1) The aqueous acrylic polyol is an acrylic polyol, which is modified to be aqueous.

The acrylic polyol has, without any limitation, for example, at least two hydroxyl groups in one molecule and is obtained by copolymerizing a (meth)acrylic monomer having a hydroxyl group and a (meth)acrylic monomer having no hydroxyl group.

Examples of the (meth)acrylic monomer having a hydroxyl group include (meth)acrylic acid esters having a hydroxyl group, such as 2-hydroxyethyl (meth)acrylate, 2-hydroxypropyl (meth)acrylate, 2-hydroxybutyl (meth)acrylate, alkylene glycol mono(meth)acrylate, and polyalkylene glycol mono(meth)acrylate. These (meth)acrylic monomers having a hydroxyl group may be used individually or in combination of two or more of them.

Examples of the (meth)acrylic monomer having no hydroxyl group include: (meth)acrylic unsaturated carboxylic acids such as (meth)acrylic acid; (meth)acrylic acid ester such as methyl (meth)acrylate, ethyl (meth)acrylate, propyl (meth)acrylate, isopropyl (meth)acrylate, butyl (meth)acrylate, isobutyl (meth)acrylate, pentyl (meth)acrylate, hexyl (meth)acrylate, 2-ethylhexyl (meth)acrylate, cyclohexyl (meth)acrylate, octyl (meth)acrylate, and decyl (meth)acrylate; and another (meth)acrylic monomer such as (meth)acrylonitrile, and (meth)acrylamide. These (meth)acrylic monomers having no hydroxyl group may be used individually or in combination of two or more of them. In the present invention, (meth)acrylic acid means acrylic acid and/or methacrylic acid.

Further, in addition to the (meth)acrylic monomer, the acrylic polyol may contain another monomer component which has a hydroxyl group and/or another monomer component which has no hydroxyl group, as long as they do not impair the effects of the present invention. Examples of another monomer component which has a hydroxyl group include unsaturated alcohols such as 3-methyl-3-butene-1-ol, 3-methyl-2-butene-1-ol, 2-methyl-3-butene-2-ol, 2-methyl-2-butene-1-ol, 2-methyl-3-butene-1-ol, and allyl alcohol.

Examples of another monomer component which has no hydroxyl group include: aromatic vinyl compounds such as styrene and  $\alpha$ -methyl styrene; and ethylenically unsaturated carboxylic acids such as maleic acid and itaconic acid. These other monomer components may be used individually or in combination of two or more of them.

A method for modifying the acrylic polyol to be aqueous includes, without any limitation, for example, a method in which a monomer such as an unsaturated carboxylic acid having a carboxyl group like (meth)acrylic acid and maleic acid is copolymerized, and the carboxyl group is neutralized with a base, thereby modifying the acrylic polyol to be aqueous, or a method in which a (meth)acrylic monomer having a

hydroxyl group is subjected to the emulsion-polymerization in the presence of an emulsifier, thereby modifying the acrylic polyol to be aqueous.

The hydroxyl value of (a-1) the aqueous acrylic polyol is preferably 50 mg KOH/g or more, and more preferably 60 mg KOH/g or more, and even more preferably 70 mg KOH/g or more, and is preferably 150 mg KOH/g or less, and more preferably 140 mg KOH/g or less, and even more preferably 130 mg KOH/g or less. If the hydroxyl value of (a-1) the aqueous acrylic polyol falls within the above range, the gloss of the paint film can be further improved. In addition, the hardness and water-resistance of the paint film can be improved. In the present invention, the hydroxyl value can be measured by using, for example, an acetylation method, in accordance with JIS K 1557-1.

The glass transition temperature of (a-1) the aqueous acrylic polyol is preferably 20° C. or more, and more preferably 22° C. or more, and even more preferably 25° C. or more, and is preferably 60° C. or less, and more preferably 57° C. or less, and even more preferably 55° C. or less. If the glass transition temperature of (a-1) the aqueous acrylic polyol falls within the above range, the production of the aqueous paint becomes easy. Further, the impact-resistance of the paint film can be enhanced.

The weight average molecular weight of (a-1) the aqueous acrylic polyol is preferably 3,000 or more, and more preferably 5,000 or more, and even more preferably 8,000 or more, and is preferably 50,000 or less, and more preferably 45,000 or less, and even more preferably 40,000 or less. If the weight average molecular weight of (a-1) the aqueous acrylic polyol falls within the above range, the water-resistance and impact-resistance of the paint film can be enhanced. The weight average molecular weight of (a-1) the aqueous acrylic polyol can be measured, for example, by gel permeation chromatography (GPC), using polystyrene as a standard material, tetrahydrofuran as an eluate, and an organic solvent system GPC columns (for example, by using "Shodex (registered trademark) KF series" available from Showa Denko K.K.).

Further, the average number (average hydroxyl group number) of hydroxyl groups contained in a molecule of (a-1) the aqueous acrylic polyol is preferably 5 or more, and more preferably 10 or more, and even more preferably 20 or more, and is preferably 100 or less, and more preferably 50 or less, and even more preferably 40 or less. If the average hydroxyl group number of (a-1) the aqueous acrylic polyol is 5 or more, because of the high reactivity with (B) the aqueous polyisocyanate, a tough paint film can be formed and the adhesion to the surface of the golf ball body becomes better. If the average hydroxyl group number is 100 or less, the water-resistance of the paint film formed becomes good. It is noted that the average hydroxyl group number of (a-1) the aqueous acrylic polyol can be calculated based on the hydroxyl value and the weight average molecular weight.

(a-1) The aqueous acrylic polyol is preferably used in the form of an aqueous liquid in which (a-1) the aqueous acrylic polyol is dissolved or dispersed in water. For example, when the aqueous liquid in which (a-1) the aqueous acrylic polyol is dissolved or dispersed in water is used, the content (non-volatile content) of (a-1) the aqueous acrylic polyol component in the aqueous liquid is preferably 20 mass % or more, more preferably 25 mass % or more, even more preferably 30 mass % or more, and is preferably 70 mass % or less, more preferably 65 mass % or less, and even more preferably 60 mass % or less. If the content of (a-1) the aqueous acrylic polyol component in the aqueous liquid falls within the above range, (a-1) the aqueous acrylic polyol can be easily mixed with (a-2) the aqueous urethane polyol or the like, thereby

facilitating the preparation of (A) the aqueous polyol composition. A method for measuring the non-volatile content will be described later.

Specific examples of (a-1) the aqueous acrylic polyol include an aqueous acrylic polyol (hydroxyl value: 108 mg KOH/g, glass transition temperature: 46° C.) available from SHINTO PAINT CO., LTD., and trade names "Bayhydrol (registered trademark) VPLS2058", "Bayhydrol (registered trademark) VPLS2235", available from Sumika Bayer Urethane Co., Ltd.

#### (1-2) Aqueous Urethane Polyol

Next, (a-2) the aqueous urethane polyol contained in (A) the aqueous polyol composition will be described.

(a-2) The aqueous urethane polyol is an aqueous compound having a plurality of urethane bonds in its molecule, and having at least two hydroxyl groups in a molecule thereof. (a-2) The aqueous urethane polyol is, for example, a hydroxyl group terminated urethane prepolymer, which is obtained by reaction between a polyisocyanate component and an aqueous polyol component such as an aqueous polyester polyol and an aqueous polyether polyol, under a condition that the hydroxyl groups of the aqueous polyol component is excessive to the isocyanate groups of the polyisocyanate component.

The aqueous polyester polyol which can constitute (a-2) the aqueous urethane polyol may be any one of a water-soluble polyester polyol or a water-dispersible polyester polyol. For example, a polyester polyol having a carboxyl group, a polyester polyol having a sulfonic group, and the like may be used as the aqueous polyester polyol. As the aqueous polyester polyol, an aqueous polyester polyol having a carboxyl group is particularly preferable, and is modified to be aqueous by neutralizing the carboxyl group thereof with a base.

The aqueous polyester polyol having a carboxyl group may be synthesized in a known method for synthesizing a polyester polyol, and can be obtained through, for example, polycondensation of a low molecular weight polyol and a polybasic acid. Further, the carboxyl group used for modifying the polyester polyol to be aqueous can be introduced from any one of the low molecular weight polyol or the polybasic acid.

The low molecular weight polyol may be any polyol publicly known for being used in the synthesis of polyester polyols, and examples thereof include: diols such as ethylene glycol, propylene glycol, 1,3-propanediol, 1,4-butanediol, 1,5-pentanediol, 3-methyl-1,5-pentanediol, 1,6-hexanediol, neopentyl glycol, diethylene glycol, triethylene glycol, tetraethylene glycol, dipropylene glycol, tripropylene glycol, 1,4-cyclohexanediol, bisphenol A; and triols such as trimethylol propane and glycerin. Examples of the low molecular weight polyol for introducing the carboxyl group in the polyester polyol include dimethylol propionic acid, dimethylol butanoic acid, dihydroxy propionic acid, and dihydroxysuccinic acid. These low molecular weight polyols may be used individually or in combination of two or more types thereof.

The polybasic acid may be any polybasic acid publicly known for being used in the synthesis of polyester polyols, and examples thereof include dibasic acids such as succinic acid, adipic acid, azelaic acid, sebacic acid, dodecanedicarboxylic acid, maleic anhydride, fumaric acid, 1,3-cyclopentanedicarboxylic acid, 1,4-cyclohexanedicarboxylic acid, terephthalic acid, isophthalic acid, 1,4-naphthalenedicarboxylic acid, 2,5-naphthalenedicarboxylic acid, 2,6-naphthalenedicarboxylic acid, naphthalic acid, and biphenyldicarboxylic acid. Examples of the polybasic acid for enabling introduction of the carboxyl group in the polyester polyol include trimellitic anhydride, and pyromellitic anhydride.

These polybasic acids may be used individually or in combination of two or more types thereof.

The aqueous polyether polyol component which can constitute (a-2) the aqueous urethane polyol preferably includes, for example, polyethylene glycol. The aqueous polyether polyol is modified to be aqueous by simply mixing it with water and stirring them. Further, the polyether polyol may be dissolved while being heated, as necessary.

The polyisocyanate component which can constitute (a-2) the aqueous urethane polyol is not limited, as long as it has at least two isocyanate groups. Examples of the polyisocyanate include an aromatic polyisocyanate such as 2,4-tolylene diisocyanate, 2,6-tolylene diisocyanate, a mixture of 2,4-tolylene diisocyanate and 2,6-tolylene diisocyanate (TDI), 4,4'-diphenylmethane diisocyanate (MDI), 1,5-naphthylene diisocyanate (NDI), 3,3'-bitolylene-4,4'-diisocyanate (TODD), xylylene diisocyanate (XDI), tetramethylxylylene-diisocyanate (TMXDI), para-phenylene diisocyanate (PPDI); an alicyclic polyisocyanate or aliphatic polyisocyanate such as 4,4'-dicyclohexylmethane diisocyanate (H<sub>12</sub>MDI), hydrogenated xylylenediisocyanate (H<sub>6</sub>XDI), hexamethylene diisocyanate (HDI), isophorone diisocyanate (IPDI), and norbornene diisocyanate (NBDI). These may be used either alone or as a mixture of at least two of them.

The hydroxyl value of (a-2) the aqueous urethane polyol is preferably 50 mg KOH/g or more, more preferably 60 mg KOH/g or more, even more preferably 70 mg KOH/g or more, and is preferably 500 mg KOH/g or less, more preferably 450 mg KOH/g or less, 400 mg KOH/g or less. If the hydroxyl value of (a-2) the aqueous urethane polyol falls within the above range, it would be possible to further improve the adhesion of the paint film to the golf ball body.

The weight average molecular weight of (a-2) the aqueous urethane polyol is preferably 200 or more, and more preferably 250 or more, and even more preferably 300 or more, and is preferably 50,000 or less, and more preferably 45,000 or less, and even more preferably 40,000 or less. If the weight average molecular weight of (a-2) the aqueous urethane polyol falls within the above range, the water-resistance and impact-resistance of the paint film can be enhanced. The weight average molecular weight of (a-2) the aqueous urethane polyol can be measured, for example, by gel permeation chromatography (GPC), using polystyrene as a standard material, tetrahydrofuran as an eluate, and an organic solvent system GPC columns (for example, by using "Shodex (registered trademark) KF series" available from Showa Denko K.K.).

Further, the average number of hydroxyl groups (average hydroxyl group number) contained in one molecule of (a-2) the aqueous urethane polyol is preferably 1.0 or more, more preferably 1.5 or more, even more preferably 2 or more, and is preferably 50 or less, and more preferably 45 or less, and even more preferably 40 or less. If the average number of hydroxyl group of (a-2) the aqueous urethane polyol is 1.0 or more, reactivity to (B) the aqueous polyisocyanate is high and thus a tough paint film can be formed and the adhesion to the surface of the golf ball body becomes better. If the average hydroxyl group number is 50 or less, the water-resistance of the paint film formed becomes better. The average hydroxyl group number of (a-2) the aqueous urethane polyol can be calculated based on the hydroxyl value and the weight average molecular weight.

(a-2) The aqueous urethane polyol is preferably used in the form of an aqueous liquid in which (a-2) the aqueous urethane polyol is dissolved or dispersed in water. For example, if an aqueous liquid in which (a-2) the aqueous urethane polyol is dissolved or dispersed in water is used, the content (non-

volatile content) of (a-2) the aqueous urethane polyol component in the aqueous liquid is preferably 20 mass % or more, more preferably 23 mass % or more, even more preferably 25 mass % or more, and is preferably 95 mass % or less, more preferably 93 mass % or less, even more preferably 90 mass % or less. If the content of (a-2) the aqueous urethane polyol component in the aqueous liquid falls within the above range, (a-2) the aqueous urethane polyol can be easily mixed with (a-1) the aqueous acrylic polyol or the like, thereby facilitating the preparation of (A) the aqueous polyol composition. A method for measuring the non-volatile content will be described later.

Specific examples of the aqueous liquid of (a-2) the aqueous urethane polyol include trade names "FLEXOREZ (registered trademark) UD-350W" and "FLEXOREZ (registered trademark) UD-320" available from King Industries, Inc., and trade name "Bayhydrol (registered trademark) VPLS2056" available from Sumika Bayer Urethane Co., Ltd. (1-3) Aqueous Urethane Resin

Next, (a-3) the aqueous urethane resin contained in (A) the aqueous polyol composition will be described.

(a-3) The aqueous urethane resin is a polyurethane resin which is modified to be aqueous.

The polyurethane resin is not particularly limited, as long as it has a plurality of urethane bonds within the molecule. For example, the polyurethane resin can be obtained by reacting a polyisocyanate component with a high molecular weight polyol component to have urethane bonds formed within the molecule. Further, a chain extension reaction with a low molecular weight polyol, a low molecular weight polyamine, or the like is performed if necessary

Examples of the polyisocyanate component which can constitute the polyurethane resin, include polyisocyanates exemplified as being used for (a-2) the aqueous urethane polyol.

The polyol component constituting the polyurethane resin may be, without any limitation, any polyol component having a plurality of hydroxyl groups. For example, a low molecular weight polyol having a molecular weight of less than 500, or a high molecular weight polyol having a molecular weight of 500 or more may be used as the polyol component.

Examples of the low molecular weight polyol are a diol such as ethylene glycol, diethylene glycol, triethylene glycol, 1,3-butanediol, 1,4-butanediol, neopentyl glycol, 1,6-hexanediol; and a triol such as glycerin, trimethylol propane, and hexane triol. Examples of the high-molecular weight polyol include a polyether polyol such as polyoxethylene glycol (PEG), polyoxypropylene glycol (PPG), and polyoxytetramethylene glycol (PTMG); a condensed polyester polyol such as polyethylene adipate (PEA), polybutylene adipate (PBA), and polyhexamethylene adipate (PHMA); a lactone polyester polyol such as poly- $\epsilon$ -caprolactone (PCL); a polycarbonate polyol such as polyhexamethylene carbonate; and an acrylic polyol. Among them, the polyol having a weight average molecular weight of about 50 to about 2,000, in particular about 100 to about 1,000 is preferably used. The above polyols may be used alone or as a mixture of at least two of them.

The polyamine component that constitutes the polyurethane resin where necessary may include any polyamine, as long as it has at least two amino groups. The polyamine component includes an aliphatic polyamine such as ethylene-diamine, propylenediamine, and hexamethylenediamine, an aromatic polyamine such as tolylenediamine, xylylenediamine, and diaminodiphenyl methane; and an alicyclic polyamine such as diaminocyclohexyl methane, piperazine, isophoronediamine; hydrazine or derivatives thereof such as succinic acid dihydrazide, adipic acid dihydrazide, phthalic

acid dihydrazide. As the low molecular weight polyol or low molecular weight polyamine, alkanolamine such as diethanolamine, monoethanolamine can be used.

The polyurethane resin has no limitation on the constitutional embodiments thereof. Examples of the constitutional embodiments are the embodiment where the polyurethane resin consists of the polyisocyanate component and the high-molecular weight polyol component; the embodiment where the polyurethane resin consists of the polyisocyanate component, the high-molecular weight polyol component and the low-molecular weight polyol component; and the embodiment where the polyurethane resin consists of the polyisocyanate component, the high-molecular weight polyol component, the low-molecular weight polyol component, and the polyamine component; and the embodiment where the polyurethane resin consists of the polyisocyanate component, the high-molecular weight polyol component and the polyamine component.

As a method for modifying the polyurethane resin to be aqueous, for example, an ionomer type self-emulsification method or a prepolymer emulsification type phase inversion emulsification method may be used.

In the ionomer type self-emulsification method, the polyurethane resin is dissolved or dispersed in water, without using an emulsifier, by introducing an ionic group in a molecule of the polyurethane resin. The ionic group includes functional groups such as a carboxyl group or an amino group which can be ionized (but not yet ionized) and ionized functional groups where the ionizable functional group is neutralized with an inorganic metal compound or amines.

As a method for introducing the ionic group in a molecule of the polyurethane resin, a known method can be employed. For example, a method in which a polyol having an ionic group is used as a part of the polyol component, a method in which a chain extender having an ionic group is used as a part or the whole of the chain extender components, or a method in which the polyol and the chain extender each having an ionic group are used as a part of the polyol component and a part or the whole of the chain extender components, respectively, may be employed.

The polyol having the ionic group includes, for example, a polyester polyol having a carboxyl group or a polyester polyol having a sulfonic group, which are exemplified as polyols used for (a-2) the aqueous urethane polyol. Examples of the chain extender having the ionic group include low molecular weight polyols such as dimethylol propionic acid, dimethylol butanoic acid, dihydroxy propionic acid, and dihydroxysuccinic acid.

In the prepolymer emulsification type phase inversion emulsification method, a relatively low molecular weight urethane prepolymer is forced to be emulsified and dispersed by a high shear in the presence of a non-ionic emulsifier, and is thereafter subjected to chain extension reaction with a polyol component or a low molecular weight polyamine component.

Each of (a-3) the aqueous urethane resin and (a-2) the aqueous urethane polyol has a plurality of urethane bonds in its molecule. (a-2) The aqueous urethane polyol has at least two hydroxyl groups in one molecule, whereas (a-3) the aqueous urethane resin substantially has no hydroxyl group. That is, a hydroxyl value of (a-3) the aqueous urethane resin is less than or equal to 5 mg KOH/g.

The glass transition temperature of (a-3) the aqueous urethane resin is preferably 20°C. or less, more preferably 15°C. or less, and even more preferably 10°C. or less. If the glass transition temperature of (a-3) the aqueous urethane resin is 20°C. or less, the elongation of the aqueous urethane resin is increased, and the tensile property of the paint film is

enhanced. The lower limit of the glass transition temperature of (a-3) the aqueous urethane resin is not limited, but may be -50°C. The glass transition temperature of (a-3) the aqueous urethane resin can be measured by using, for example, a dynamic viscoelasticity measurement apparatus.

The elongation of (a-3) the aqueous urethane resin is preferably 100% or more, and more preferably 150% or more, and even more preferably 200% or more, and is preferably 2,000% or less, more preferably 1,900% or less, and even more preferably 1,800% or less. If the elongation of (a-3) the aqueous urethane resin falls within the above range, the adhesion of the paint film to the surface of a golf ball body can be enhanced. The upper limit of the elongation of (a-3) the aqueous urethane resin is not limited, but may be 2,500%. The elongation of (a-3) the aqueous urethane resin can be measured by using, for example, Autograph available from SHIMADZU CORPORATION.

In the present invention, the glass transition temperature and the elongation of (a-3) the aqueous urethane resin are physical property values of the film obtained from (a-3) the aqueous urethane resin, and the measurement methods will be described later.

If a water-dispersible urethane resin is used as (a-3) the aqueous urethane resin, the volume average particle diameter of the urethane resin is preferably 50 nm or more, more preferably 55 nm or more, and even more preferably 60 nm or more, and is preferably 300 nm or less, more preferably 250 nm or less, and even more preferably 200 nm or less. If the volume average particle diameter of the dispersed urethane resin falls within the above range, the gloss of the paint film can be enhanced. The volume average particle diameter of the urethane resin dispersed in water can be measured by using a laser diffraction/scattering type particle size distribution measurement apparatus.

(a-3) The aqueous urethane resin is preferably used in the form of an aqueous liquid in which (a-3) the aqueous urethane resin is dissolved or dispersed in water. For example, when an aqueous liquid in which (a-3) the aqueous urethane resin is dispersed in water is used, the content (non-volatile content) of (a-3) the aqueous urethane resin component in the aqueous liquid is preferably 10 mass % or more, more preferably 12 mass % or more, and even more preferably 15 mass % or more, and is preferably 50 mass % or less, more preferably 47 mass % or less, and even more preferably 45 mass % or less. When the content of (a-3) the aqueous urethane resin component in the aqueous liquid falls within the above range, (a-3) the aqueous urethane resin can be easily mixed with (a-1) the aqueous acrylic polyol or the like, thereby facilitating the preparation of (A) the aqueous polyol composition. A method for measuring the non-volatile content will be described later.

Specific examples of (a-3) the aqueous urethane resin include trade names "SUPERFLEX (registered trademark) 300" and "SUPERFLEX (registered trademark) 500H" available from Dai-ichi Kogyo Seiyaku Co., Ltd.

The content of (a-3) the aqueous urethane resin in (A) the aqueous polyol composition is preferably 20 mass % or more, more preferably 25 mass % or more, and even more preferably 30 mass % or more, and is preferably 80 mass % or less, more preferably 75 mass % or less, and even more preferably 70 mass % or less. If the content of (a-3) the aqueous urethane resin in (A) the aqueous polyol composition falls within the above range, the adhesion of the paint film to the surface of a golf ball body can be enhanced.

Further, as the blending ratio of (a-1) the aqueous acrylic polyol to (a-2) the aqueous urethane polyol in (A) the aqueous polyol composition (when the total is 100% by mass), (a-1)

## 11

the aqueous acrylic polyol/(a-2) the aqueous urethane polyol is preferably 40 mass % to 90 mass %/60 mass % to 10 mass %, more preferably 45 mass % to 85 mass %/55 mass % to 15 mass %, and even more preferably 50 mass % to 80 mass %/50 mass % to 20 mass %. If the blending ratio (a-1)/(a-2) falls within the above range, the gloss of the paint film which is obtained from the two-component curing type urethane-based aqueous paint of the present invention, the adhesion thereof to the golf ball body, and the durability thereof can be enhanced.

(A) The aqueous polyol composition preferably contains water as a dispersion medium. In this case, the non-volatile content in (A) the aqueous polyol composition is preferably 20 mass % or more, more preferably 25 mass % or more, and even more preferably 30 mass % or more, and is preferably 85 mass % or less, more preferably 80 mass % or less, and even more preferably 75 mass % or less. If the non-volatile content in (A) the aqueous polyol composition is 20 mass % or more, reactivity between (A) the aqueous polyol composition and (B) the aqueous polyisocyanate described below becomes good. Further, if the non-volatile content in (A) the aqueous polyol composition is 85 mass % or less, the viscosity is not excessively high, and the painting becomes good. A method for measuring the non-volatile content will be described below.

## (1-4) Aqueous Polyisocyanate

(B) The aqueous polyisocyanate will be described. (B) The aqueous polyisocyanate is not limited, as long as it is any modified product obtained by modifying the polyisocyanate component to be aqueous (water-soluble, or water-dispersible). For example, (B) the aqueous polyisocyanate may be an aqueous polyisocyanate obtained by modifying a polyisocyanate component with polyoxyalkylene ether alcohol.

The polyisocyanate component constituting the aqueous polyisocyanate includes, for example, an aromatic polyisocyanate such as 2,4-tolylene diisocyanate, 2,6-tolylene diisocyanate, a mixture (TDI) of 2,4-tolylene diisocyanate and 2,6-tolylene diisocyanate, 4,4'-diphenylmethane diisocyanate (MDI), 1,5-naphthylene diisocyanate (NDI), 3,3'-bitolylene-4,4'-diisocyanate (TODI), xylylene diisocyanate (XDI), tetramethylxylylenediisocyanate (TMXDI) and para-phenylene diisocyanate (PPDI); and an alicyclic or aliphatic polyisocyanate such as 4,4'-dicyclohexylmethane diisocyanate ( $H_{12}$ MDI), hydrogenated xylylenediisocyanate ( $H_6$ XDI), hexamethylene diisocyanate (HDI), isophorone diisocyanate (IPDI), norbornene diisocyanate (NBDI) and derivatives thereof.

Examples of the derivative of the polyisocyanate include: isocyanurate of diisocyanate; an adduct obtained through reaction between a diisocyanate and a low molecular weight triol such as trimethylolpropane or glycerin (it is preferable that a free diisocyanate is removed); an allophanate-modified product; and a biuret-modified product. One example of the allophanate-modified product is a trifunctional polyisocyanate which is obtained by further reacting a diisocyanate with a urethane bond formed through a reaction between a diisocyanate and a low molecular weight diol. One example of the biuret-modified products is a trifunctional polyisocyanate which is obtained by further reacting a diisocyanate with a urea bond formed through a reaction between a diisocyanate and a low molecular weight diamine. The polyisocyanates and the derivatives thereof may be used individually or in combination of two or more types.

(B) The aqueous polyisocyanate preferably contains, as a polyisocyanate component, (b-1) hexamethylene diisocyanate and/or a derivative thereof, and (b-2) isophorone diisocyanate and/or a derivative thereof. (B) The aqueous polyiso-

## 12

cyanate more preferably consists of (b-1) hexamethylene diisocyanate and/or a derivative thereof and (b-2) isophorone diisocyanate and/or a derivative thereof. According to this embodiment, the weather-resistance of the paint film obtained from the two-component curing type urethane-based aqueous paint of the present invention is enhanced.

As (b-1) the hexamethylene diisocyanate and/or a derivative thereof, an isocyanurate of hexamethylene diisocyanate is preferable. Further, as (b-2) the isophorone diisocyanate and/or a derivative thereof, an isocyanurate of isophorone diisocyanate is preferable.

As the blending ratio of (b-1) the hexamethylene diisocyanate and/or a derivative thereof, to (b-2) the isophorone diisocyanate and/or a derivative thereof in (B) the aqueous polyisocyanate (when the total is 100% by mass), (b-1) the hexamethylene diisocyanate and/or a derivative thereof/(b-2) the isophorone diisocyanate and/or a derivative thereof is preferably 50 mass % to 99 mass %/50 mass % to 1 mass %, more preferably 55 mass % to 95 mass %/45 mass % to 5 mass %, and even more preferably 60 mass % to 90 mass %/40 mass % to 10 mass %. If the blending ratio ((b-1)/(b-2)) falls within the above range, the adhesion of the paint film obtained from the two-component curing type urethane-based aqueous paint of the present invention to a golf ball body, and the durability thereof can be enhanced.

Specific examples of (B) the aqueous polyisocyanate include trade name "CR-60N" available from DIC Corporation, trade names "CORONATE (registered trademark) C3062, C3053" available from NIPPON POLYURETHANE INDUSTRY CO., LTD., trade names "Bayhydur (registered trademark) 3100" and "Bayhydur (registered trademark) 401-70" available from Sumika Bayer Urethane Co., Ltd., trade name "1-3" available from SHINTO PAINT CO., LTD., and trade name "WG-6B" available from Wayaku Paint Co., Ltd.

## (1-5) Other Details for Two-Component Curing Type Urethane-Based Aqueous Paint

In the two-component curing type urethane-based aqueous paint according to the present invention, the molar ratio (NCO/OH) of the isocyanate group (NCO) of (B) the aqueous polyisocyanate to the hydroxyl group (OH) of (A) the aqueous polyol composition is preferably 1.25 or more, and is preferably 2.50 or less. If the molar ratio (NCO/OH) is less than 1.25, the amount of the isocyanate groups is too small, and leveling effect cannot be obtained. Therefore, the appearance of the obtained paint film may deteriorate. Further, if the molar ratio (NCO/OH) is more than 2.50, the amount of the isocyanate groups is excessive, and the appearance of the obtained paint film may deteriorate as well as the obtained paint film may be hard and fragile. The appearance of the obtained paint film deteriorates because an excessive amount of isocyanate groups in the paint may promote a reaction between the moisture in the air and the isocyanate groups, thereby generating a lot of carbon dioxide gas. The molar ratio (NOC/OH) is preferably 1.25 or more, more preferably 1.30 or more, and is preferably 2.5 or less, more preferably 2.4 or less.

The two-component curing type urethane-based aqueous paint of the present invention may contain, in addition to the components described above, additives, such as a pigment, an ultraviolet absorber, an antioxidant, a light stabilizer, a fluorescent brightener, an anti-blocking agent, a leveling agent, a slip agent, and a viscosity modifier, which are generally contained in the paint for a golf ball, as necessary.

The viscosity of the two-component curing type urethane-based aqueous paint of the present invention is preferably 50 mPa·s or more, more preferably 60 mPa·s or more, even more

preferably 70 mPa·s or more, and is preferably 350 mPa·s or less, more preferably 340 mPa·s or less, 330 mPa·s or less. If the viscosity is 50 mPa·s or more, the paint applied on the surface of the golf ball body does not sag, and the paint film having the even thickness to the higher extent can be obtained, and if the viscosity is 350 mPa·s or less, spraying becomes good and thus, the appearance (gloss) of the painted golf ball becomes better in the case of spraying the paint with an air gun. The method of measuring the viscosity of the two-component curing type urethane-based aqueous paint will be described later.

In the present invention, the change in the viscosity of the two-component curing type urethane-based aqueous paint used in the present invention is within the rise by about 10 mPa·s within 2 hours after (A) the aqueous polyol composition and (B) the aqueous polyisocyanate are mixed. Thus, the processability is not lowered in the case that (A) the aqueous polyol composition and (B) the aqueous polyisocyanate are mixed little by little.

#### (2) Method for Producing Golf Ball

Next, the applying method of the two-component curing type urethane-based aqueous paint used in the present invention will be described.

##### (2-1) Method I

In one preferable embodiment, the method for producing the golf ball of the present invention comprises applying a two-component curing type urethane-based aqueous paint containing (A) an aqueous polyol composition and (B) an aqueous polyisocyanate to a golf ball body having a surface temperature ranging from 30° C. to 80° C.

The surface temperature of the golf ball body ranges from 30° C. to 80° C. when applying the two-component curing type urethane-based aqueous paint. If the surface temperature of the golf ball body when applying the paint is less than 30° C., the sagging of the applied paint is not sufficiently suppressed, thus the improved effect of the even thickness of the paint film is not obtained. If the surface temperature is more than 80° C., the vaporizing rate of the water contained in the paint becomes too high, it becomes difficult to defoam the paint, the leveling is bad, and the gloss of the obtained paint film is lowered. The surface temperature of the golf ball body when applying the paint is preferably 33° C. or more, more preferably 40° C. or more, even more preferably 45° C. or more, and is preferably 80° C. or less, more preferably 75° C. or less.

The method of adjusting the temperature of the golf ball includes, without limitation, for example, putting the golf ball into the oven set at the predetermined temperature, irradiating microwaves, or irradiating infrared light.

The temperature of the two-component curing type urethane-based aqueous paint when applying it to the golf ball body is preferably 10° C. or more, more preferably 15° C. or more, even more preferably 20° C. or more, and is preferably 50° C. or less, more preferably 45° C. or less, even more preferably 40° C. or less. If the temperature of the two-component curing type urethane-based aqueous paint is 10° C. or more, the viscosity of the paint is lowered, and thus the processability of the paint becomes better. If the temperature is 50° C. or less, the lowering of the pot life of the paint can be suppressed.

##### (2-2) Method II

In another preferable embodiment, the method for producing the golf ball of the present invention comprises

overpainting a two-component curing type urethane-based aqueous paint containing (A) the aqueous polyol composition and (B) the aqueous polyisocyanate to a golf ball body mul-

iple times until a paint film has a desired thickness, such that an applied amount (dry mass) of the paint per one time ranges from 5 mg below 80 mg.

If the applied amount (dry mass) of the paint per one time is less than 5 mg for each golf ball, the applying times required to reach a desired film thickness become too much, thereby causing reduction of productivity. On the other hand, if the applied amount (dry mass) of the paint per one time is 80 mg or more for each golf ball, the amount of the paint to be sprayed in one painting step is too much to control the sagging of the paint that has been applied, thereby lowering the evenness of the film thickness of the obtained paint film. The applied amount (dry mass) of the paint per one time is preferably 10 mg or more, and more preferably 15 mg or more, and is preferably 75 mg or less, more preferably 70 mg or less.

The thickness of the paint film obtained by applying and drying the paint in one operation is preferably 2 μm or more, and more preferably 3 μm or more, and even more preferably 4 μm or more, and is preferably 10 μm or less, more preferably 9 μm or less, and even more preferably 8 μm or less.

The times of overpainting the paint are preferably, without limitation, at least two times, and should be changed depending upon the desired film thickness. For example, if the desired film thickness ranges from 10 μm to 20 μm, the overpainting times are preferably 4 times or less, and more preferably 3 times or less. If the overpainting times are 4 times or less, the applied amount of the paint per one time is not excessively small, thereby enhancing the evenness of the film thickness of the obtained paint film. In light of workability, the overpainting times are particularly preferable 2 times.

The painting interval in the overpainting operation is preferably longer than 0 second and is preferably 20 seconds or less. The painting interval is an interval time between each painting operation, that is, a flash-off time. In other words, if the overpainting times are 2 times, an interval time from the end of the first painting operation to the start of the second painting operation is preferably longer than 0 second and is preferably 20 seconds or less. If the painting interval in the overpainting operation falls within the above range, the evenness of the obtained paint film is further improved. The painting interval is preferably 1 second or more, more preferably 2 seconds or more, and is preferably 15 seconds or less, more preferably 10 seconds or less.

Further, in the case of overpainting the paint multiple times, it is also preferable that the paint is applied after the paint having been previously applied to the golf ball body is dried. In this case, the temperature for drying the paint having been previously applied is preferably 30° C. or higher, more preferably 40° C. or higher, and even more preferably 50° C. or higher, and is preferably 80° C. or lower, more preferably 70° C. or lower, and even more preferably 60° C. or lower. Further, the drying time is preferably 1 hour or longer, and more preferably 2 hours or longer, and even more preferably 3 hours or longer.

An ambient temperature at which the paint is applied is not limited and preferably ranges from 20° C. to 27° C. Further, an ambient humidity at which the paint is applied is not limited and is preferably 65% or less. The paint finally obtained by overpainting may be dried, for example, at a temperature ranging from 30° C. to 70° C. for 1 to 24 hours.

##### (2-3) Other Details for Method I and Method II

The method of applying the two-component curing type urethane-based aqueous paint is not limited, and includes a conventional method for the two-component mixing type paint. For example, (A) the aqueous polyol composition and (B) the aqueous polyisocyanate are mixed, and then applied to the golf ball with an air gun or in the electrostatic coating

## 15

method. Among them, the use of the air gun is preferable in view of obtaining the paint film with the higher degree of the evenness.

In the case of applying the paint with the air gun, (A) the aqueous polyol composition and (B) the aqueous polyisocyanate can be mixed little by little for use, or (A) the aqueous polyol composition and (B) the aqueous polyisocyanate are fed with the respective pumps and continuously mixed in a constant ratio through the line mixer such as the static mixer located in the stream line just before the air gun. Alternatively, (A) the aqueous polyol composition and (B) the aqueous polyisocyanate can be air-sprayed respectively with the spray gun having the device for controlling the mixing ratio thereof.

In the case of using an air gun, a spray distance, that is, a minimum distance between the spray nozzle of the air gun and the surface of a golf ball body, is preferably 5 cm or more, and more preferably 6 cm or more, and is preferably 15 cm or less, and more preferably 14 cm or less. If the spray distance is 5 cm or longer, the evenness of the film thickness of the obtained paint film can be enhanced. If the spray distance is 15 cm or less, it is possible to prevent the paint from spreading without being applied to the golf ball body.

A spraying air pressure of the air gun is preferably 0.01 MPa or more, and more preferably 0.05 MPa or more, and is preferably 0.30 MPa or less, and more preferably 0.25 MPa or less. If the spraying air pressure is 0.01 MPa or more, the paint can be fully atomized, thereby enhancing the evenness of the paint film. If the spraying air pressure is 0.30 MPa or less, a blast of air discharged from the air gun is not excessively strong, and it is possible to prevent the golf ball from falling from a supporter (rotating element) by air.

The air pressure for the air gun from the compressed air tank is preferably 0.01 MPa or more, more preferably 0.05 MPa or more, and is preferably 0.30 MPa or less, and more preferably 0.25 MPa or less. If the air pressure of the compressed air tank is 0.01 MPa or more, the paint can be fully atomized, thereby enhancing the evenness of the paint film. If the air pressure of the compressed air tank is 0.30 MPa or less, a blast of air discharged from the air gun is not excessively strong, and it is possible to prevent the golf ball from falling from the supporter (rotating element) by air.

The spraying air pressure of the air gun is an air pressure at the nozzle of the air gun, and the air pressure of the compressed air tank is a pressure of the air supplied to the air gun.

Further, in the case of using an air gun, painting time at one time is preferably 0.1 second or longer, and more preferably 0.5 second or longer, and is preferably 3 seconds or less, and more preferably 2.5 seconds or less. If the painting time at one time is 0.1 second or longer, a blast of air discharged from the air gun is not excessively strong, and it is possible to prevent the golf ball body from falling from the supporter (rotating element) by air. On the other hand, if the painting time is 3 seconds or less, a blast of air discharged from the air gun is not excessively weak, and the paint can be fully atomized, thereby enhancing the evenness of the paint film.

A manner in which the painting is performed by using the air gun is not limited, for example, and includes a manner shown in FIG. 1. FIG. 1 is a schematic diagram illustrating an exemplary painting manner using an air gun. The manner of painting includes supporting the golf ball 2 with the three prongs 3a to 3c, which are set up on a horizontally rotatable rotating element 1, rotating the rotating element 1 while supporting the golf ball 2, spacing a spray distance between the spray gun 4 and the golf ball 2, and spraying an atomized paint while moving the air gun 4 in up and down direction. In this case, the rotation speed of the rotating element 1 is preferably

## 16

300 rpm or more, and more preferably 400 rpm or more, and is preferably 800 rpm or less, and more preferably 700 rpm or less.

The two-component curing type urethane-based aqueous paint applied to the golf ball body is dried at the temperature from 30° C. to 70° C. for 1 hour to 24 hours to form a paint film.

The thickness of the paint film after drying is preferably, without limitation, 4 µm or more, more preferably 5 µm or more, and is preferably 50 µm or less, more preferably 40 µm or less. If the thickness is less than 4 µm, the paint film is likely to wear off due to the continued use. If the thickness is more than 50 µm, the effect of the dimples is lowered, and thus the flying performance of the golf ball tends to be low. The paint film preferably has a single-layered structure. If the paint film has a single-layered structure, the process of applying the paint is simplified. In the present invention, the paint film shows the excellent property even if it has the single-layered structure. The paint film is preferably an outermost clear paint layer.

## (3) Painted Golf Ball

The golf ball of the present invention is a painted golf ball that comprises a golf ball body and a paint film, and is produced by the method of the present invention.

The golf ball body does not have no limitation on the structure, and may be a one-piece golf ball, a two-piece golf ball, a multi-piece golf ball including a three-piece-golf ball, or a wound golf ball. The present invention can be applied appropriately to any one of the above golf ball.

Examples of the cover material constituting the cover include, various resins such as an ionomer resin, a polyester resin, polyurethane resins like a thermoplastic urethane resin and a thermosetting urethane resin, and a polyamide resin; and various thermoplastic elastomers such as a thermoplastic polyamide elastomer having a trade name "Pebax (registered trademark)" (e.g. "Pebax 2533") commercially available from Arkema Inc., a thermoplastic polyester elastomer having a trade name "Hytrell (registered trademark)" (e.g. "Hytrell 3548" and "Hytrell 4047") commercially available from DuPont-Toray Co., Ltd., a thermoplastic polyurethane elastomer having a trade name "Elastollan (registered trademark)" (e.g. "Elastollan XNY97A") available from BASF Japan Ltd, and thermoplastic polystyrene elastomers having a trade name "Rabalon (registered trademark)" (e.g. "Rabalon T3221C") and having a trade name "Primalloy" commercially available from Mitsubishi Chemical Corporation, and the like. These resin components may be used solely or in combination of two or more types thereof.

The cover in the present invention may contain a pigment component such as a white pigment (titanium oxide), a blue pigment, a red pigment, and the like, a specific gravity adjusting agent such as zinc oxide, calcium carbonate, barium sulfate, and the like, a dispersant, an antioxidant, an ultraviolet absorber, a light stabilizer, a fluorescent material or a fluorescent brightener, and the like as long as they do not impair the performance of the cover.

An embodiment for molding a cover is not particularly limited, and includes an embodiment which comprises injection molding the cover composition directly onto the core, or an embodiment which comprises molding the cover composition into a hollow-shell, covering the core with a plurality of the hollow-shells and subjecting the core with a plurality of the hollow shells to the compression-molding (preferably an embodiment which comprises molding the cover composition into a half hollow-shell, covering the core with the two half hollow-shells, and subjecting the core with the two half hollow-shells to the compression-molding).

In the case of directly injection molding the cover composition onto the core, it is preferred to use upper and lower molds for forming a cover having a spherical cavity and pimples, wherein a part of the pimple also serves as a retractable hold pin. When forming the cover by injection molding, the hold pin is protruded to hold the core, and the cover composition which has been heated and melted is charged and then cooled to obtain a cover. For example, the cover composition heated and melted at the temperature of 150° C. to 230° C. is charged into a mold held under the pressure of 980 KPa to 1,500 KPa for 0.1 to 1 second. After cooling for 15 to 60 seconds, the mold is opened and the golf ball with the cover molded is taken out from the mold.

When molding the cover in a compression molding method, molding of the half shell can be performed by either compression molding method or injection molding method, and the compression molding method is preferred. The compression-molding of the cover composition into half shell can be carried out, for example, under a pressure of 1 MPa or more and 20 MPa or less at a temperature of -20° C. or more and 70° C. or less relative to the flow beginning temperature of the cover composition. By performing the molding under the above conditions, a half shell having a uniform thickness can be formed. Examples of a method for molding the cover using half shells include compression molding by covering the core with two half shells. The compression molding of half shells into the cover can be carried out, for example, under a pressure of 0.5 MPa or more and 25 MPa or less at a temperature of -20° C. or more and 70° C. or less relative to the flow beginning temperature of the cover composition. By performing the molding under the above conditions, a cover for a golf ball having a uniform thickness can be formed.

The molding temperature means the highest temperature where the temperature at the surface of the concave portion of the lower mold reaches from closing through opening the molds. Further, the flow beginning temperature of the cover material can be measured in a pellet form with the following conditions by using a flow characteristics evaluation apparatus (Flow Tester CFT-500D, manufactured by Shimadzu Corporation).

Measuring conditions: Area size of a plunger: 1 cm<sup>2</sup>, Die length: 1 mm, Die diameter: 1 mm, Load: 588.399 N, Start temperature: 30° C., and Temperature increase rate: 3° C./min.

When molding a cover, the concave portions called "dimple" are usually formed on the surface. The total number of the dimples formed on the cover is preferably 200 or more and 500 or less. If the total number is less than 200, the dimple effect is hardly obtained. On the other hand, if the total number exceeds 500, the dimple effect is hardly obtained because the size of the respective dimples is small. The shape (shape in a plan view) of dimples includes, for example, without limitation, a circle, polygonal shapes such as roughly triangular shape, roughly quadrangular shape, roughly pentagonal shape, and roughly hexagonal shape, another irregular shape. The shape of the dimples is employed solely or in combination at least two of them. After the cover is molded, the mold is opened and the golf ball body is taken out from the mold, and as necessary, the golf ball body is preferably subjected to surface treatments such as deburring, cleaning, and sandblast. If desired, a paint film or a mark may be formed.

Next, the core used for the wound golf ball, two-piece golf ball, multi-piece golf ball, and the one-piece golf ball body will be explained.

As the core or the one-piece golf ball body, a conventionally known rubber composition (hereinafter simply referred to as "core rubber composition" occasionally) may be employed, and they can be molded by, for example, heat-pressing a rubber composition containing a diene rubber as a base rubber, a crosslinking initiator, and a co-crosslinking agent.

As the diene rubber, typically preferred is the high cis-polybutadiene having cis-1,4-bond in a proportion of 40% or more, more preferably 70% or more, even more preferably 90% or more in view of its superior repulsion property. The co-crosslinking agent includes; for example,  $\alpha,\beta$ -unsaturated carboxylic acid having 3 to 8 carbon atoms or a metal salt thereof, more preferably a metal salt of acrylic acid or methacrylic acid. As the metal constituting the metal salt, for example, zinc, magnesium, calcium, aluminum and sodium may be used, and among them, zinc is preferred. The amount of the co-crosslinking agent to be used is preferably 20 parts or more, and is preferably 50 parts or less. As the crosslinking initiator, an organic peroxide is preferably used. Examples of the organic peroxide for use in the present invention are dicumyl peroxide, 1,1-bis(t-butylperoxy)-3,5-trimethylcyclohexane, 2,5-dimethyl-2,5-di(t-butylperoxy)hexane, and di-t-butyl peroxide. Among them, dicumyl peroxide is preferable. An amount of the crosslinking initiator to be blended in the rubber composition is preferably 0.2 part by mass or more, more preferably 0.3 part by mass or more, and is preferably 1.5 parts by mass or less, more preferably 1.0 parts by mass or less based on 100 parts by mass of the base rubber. The core rubber composition may further contain an organic sulfur compound. As the organic sulfur compound, a diphenyl disulfide or a derivative thereof may be preferably used. The amount of the organic sulfur compound is preferably 0.1 part by mass or more, more preferably 0.3 part by mass or more, and preferably 5.0 parts by mass or less, more preferably 3.0 parts by mass or less relative to 100 parts by mass of the base rubber.

The core rubber composition may further contain a gravity adjusting agent such as zinc oxide or barium sulfate, an antioxidant, or a colored powder in addition to the base rubber, the crosslinking initiator, the co-crosslinking agent and the organic sulfur compound. The conditions for press-molding the core rubber composition should be determined appropriately depending on the rubber composition. The press-molding is preferably carried out for 10 to 60 minutes at the temperature of 130° C. to 200° C. or the press-molding is preferably carried out in a two-step heating, for example, for 20 to 40 minutes at the temperature of 130° C. to 150° C., and continuously for 5 to 15 minutes at the temperature of 160° C. to 180° C.

In the case that the golf ball of the present invention is a multi-piece golf ball including a three-piece golf ball, the material for the intermediate layer disposed between the core and the cover includes a thermoplastic resin such as a polyurethane resin, an ionomer resin, a polyamide resin, and polyethylene; and a thermoplastic elastomer such as a polystyrene elastomer, a polyolefin elastomer, a polyurethane elastomer, a polyester elastomer; and a cured product of a rubber composition. Herein, examples of the ionomer resin include one prepared by neutralizing at least a part of carboxyl groups in a copolymer composed of ethylene and  $\alpha,\beta$ -unsaturated carboxylic acid with a metal ion, and one prepared by neutralizing at least a part of carboxyl groups in a terpolymer composed of ethylene,  $\alpha,\beta$ -unsaturated carboxylic acid and  $\alpha,\beta$ -unsaturated carboxylic acid ester with a metal ion. The intermediate layer may further contain a specific gravity adjusting agent such as barium sulfate, tungsten and the like, an antioxidant, and a pigment.

## EXAMPLES

Hereinafter, the present invention will be described in detail by way of example. The present invention is not limited to examples described below. Various changes and modifications can be made without departing from the spirit and scope of the present invention.

## [Evaluation Methods]

## (1) Surface Temperature of Golf Ball Body when Applying a Paint

The surface temperature of the golf ball body when applying a paint was measured with a contact type thermometer ("ERK-2000K" available from SANWAKEIKI SEI-SAKUSHO Co., LTD.) or an infrared thermography device ("Thermo tracer TH9100MV/WV" available from NEC Avio Infrared Technologies Co., Ltd.)

## (2) Appearance of the Painted Golf Ball

The appearance of the painted golf ball was visually observed, and evaluated in accordance with the following evaluation criteria.

## Evaluation Criteria

E(Excellent): a state in which the surface was very smooth and very glossy.

G(Good): a state in which the surface was smooth and glossy.

F(Fair): a state in which the surface was slightly uneven, and was not so glossy.

P(Poor): a state in which the surface was substantially uneven, and was not glossy.

## (3) Evenness of the Film Thickness

A part of the surface of the painted golf ball was cut out to form a test piece (about 7 square millimeters) for observing the film thickness of the paint film. As to 6 dimples, the thicknesses of the paint film at the bottom and the edge, and a slope surface of each dimple were measured by using a microscope to obtain the respective averages, and the evaluation was made in accordance with the following evaluation criteria. Measuring points of the bottom and the edge, and the slope surface of each dimple will be described with reference to FIG. 2. FIG. 2 is a schematic diagram illustrating a cross-section including the bottom De of a dimple 10 and the center of a golf ball 2. The bottom De of the dimple is the deepest portion of the dimple 10. The edges Ed are tangent points at which the dimple 10 is tangent to a tangent line T which is drawn tangent to the farthest opposite ends of the dimple 10. A measurement point S on the slope surface is a point at which the slope surface of the dimple intersects the perpendicular line extending toward the dimple 10 from the center point of the straight line connecting between the bottom De and the edge Ed of the dimple.

## Evaluation Criteria

The average of the film thicknesses at the bottoms of the dimples, the average of the film thicknesses at the edges of the dimples, and the average of the film thicknesses at the slope surfaces of the dimples are represented by x, y, and z, respectively.

Good:  $|x-y| \leq 3 \mu\text{m}$  and  $|y-z| \leq 3 \mu\text{m}$  and  $|z-x| \leq 3 \mu\text{m}$

Poor:  $|x-y| > 3 \mu\text{m}$  or  $|y-z| > 3 \mu\text{m}$  or  $|z-x| > 3 \mu\text{m}$

## (4) Adhesion of Paint Film

A metal-headed driver (W#1) was installed on a swing robot manufactured by True Temper Co. Each painted golf ball was repeatedly hit at a head speed of 45 m/s 50 times, and thereafter the peeling state of the paint film was observed, and the evaluation was made in accordance with the following evaluation criteria.

## Evaluation Criteria

E(Excellent): The paint film did not peel off at all.

G(Good): An area in which the paint film peeled off was 1% or less with respect to the total area of the paint film.

F(Fair): An area in which the paint film peeled off was more than 1% and 5% or less with respect to the total area of the paint film.

P(Poor): An area in which the paint film peeled off more than 5% with respect to the total area of the paint film.

## (5) Elongation of the Aqueous Urethane Resin

An aqueous urethane resin was used to produce a film having a film thickness of 500  $\mu\text{m}$ . Drying was performed under the condition that preliminary drying was performed at room temperature for 15 hours, and final drying was per-

formed at 80° C. for 6 hours, and at 120° C. for 20 minutes. Subsequently, the obtained film was stamped out to form a test piece, and the elongation was measured with a Tensilon universal material testing Instrument. The measurement was performed under the condition that the length of the test piece was 30 mm and the crosshead speed was 200 mm/min.

## (6) Glass Transition Temperature

The glass transition temperature of the aqueous acrylic polyol was measured by using a differential scanning calorimeter (DSC) ("Q200" available from TA Instruments Inc.). The measurement was performed under the condition of the measurement temperature range: -50° C. to 200° C. and the temperature increase rate: 20° C./min.

The glass transition temperature of the aqueous urethane resin was measured by using a dynamic viscoelasticity measuring apparatus (Rheogel-E4000 available from UBM Co., Ltd.). The measurement was performed under the conditions of the oscillation frequency: 10 Hz, the measurement temperature range: -100° C. to 200° C., and the temperature increase rate: 2° C./min. A film produced by using an aqueous urethane resin was used as a test sample. The drying was performed under the condition that preliminary drying was performed at room temperature for 15 hours, and final drying was performed at 80° C. for 6 hours and at 120° C. for 20 minutes.

## (7) Non-Volatile Content

Approximately 2 g of a sample was put on an aluminum plate and was forced to be dried at 150° C. for 1 hour, and the non-volatile content was determined, based on the mass before drying and the mass after drying.

## (8) Viscosity

The viscosity of the two-component curing type urethane-based aqueous paint for a golf ball was measured by using a single cylinder rotational viscometer ("Viscotester VT-04F" available from Riontech Co., Ltd). The measurement was performed by using a rotor No. 3, and the rotation speed of the rotor was 62.5  $\text{min}^{-1}$ , and the measurement temperature was 25° C. The viscosity of the two-component curing type urethane-based aqueous paint according to the present invention was measured immediately after (A) the aqueous polyol composition and (B) the aqueous polyisocyanate were mixed.

## [Production of the Two-piece Golf Ball]

## (1) Preparation of Solid Core

The rubber composition shown in Table 1 was kneaded and heat-pressed with upper and lower molds each having a spherical cavity at the heating condition of 160° C. for 13 minutes to obtain the solid core in a spherical shape having a diameter of 39.3 mm.

TABLE 1

| Core formulation     | Amount (parts) |
|----------------------|----------------|
| Polybutadiene rubber | 100            |
| Zinc oxide           | 5.6            |
| Zinc acrylate        | 22.0           |
| Calcium carbonate    | 21.0           |
| Dicumyl peroxide     | 1.85           |

Notes on Table 1:

Polybutadiene rubber: BR-51 (cis content: 96%) available from JSR.

Zinc acrylate: "ZNDA-90S" produced by NIHON JYORYU KOGYO.

Zinc oxide: "Ginrei R" produced by Toho-Zinc.

Calcium carbonate: "BF300" produced by SHIRAI SHI CALCIUM KAISHA, LTD

Dicumyl peroxide: "Percumyl D" produced by NOF Corporation.

## (2) Preparation of the Cover Material

The materials shown in Table 2 were mixed using a twin-screw kneading extruder to obtain the cover composition in the form of pellet. The extrusion was conducted in the following conditions: screw diameter=45 mm, screw revolu-

tions=200 rpm, and screw L/D=35. The cover composition was heated to from 200° C. to 260° C. at the die position of the extruder.

TABLE 2

| Cover material | Amount (parts) |
|----------------|----------------|
| Himilan 1605   | 40             |
| Himilan 1706   | 30             |
| Himilan 1707   | 30             |
| Titanium oxide | 2              |

Notes on Table 2:

HIMILAN 1605: an ionomer resin of a sodium ion-neutralized ethylene-methacrylic acid copolymer, available from MITSUI-DUPONT POLYCHEMICAL.

HIMILAN 1706: an ionomer resin of a zinc ion-neutralized ethylene-methacrylic acid copolymer, available from MITSUI-DUPONT POLYCHEMICAL.

HIMILAN 1707: an ionomer resin of a sodium ion-neutralized ethylene-methacrylic acid copolymer, available from MITSUI-DUPONT POLYCHEMICAL.

### (3) Preparation of the Golf Ball Body

The cover composition thus prepared was directly injection-molded onto the core to form the cover, thereby obtaining the two-piece golf ball body having a diameter of 42.7 mm. The upper and lower molds for forming the cover have a spherical cavity with pimples. The part of the pimples can

serve as a hold pin which is retractable. When forming the golf ball body, the hold pins were protruded to hold the core, and the resin heated at 210° C. was charged into the mold held under the pressure of 80 tons for 0.3 seconds. After cooling for 30 seconds, the molds were opened and then the golf ball body was discharged. Dimples were formed on the surface of the golf ball.

### (4) Formation of Paint Film for Golf Balls No. 1 to No. 16

The surfaces of the obtained golf ball bodies were subjected to the sandblast treatment, and the golf ball bodies were heated by keeping them at the desired temperature for 10 minutes or more. Then, the two-component curing type aqueous urethane-based paint shown in Tables 3 and 4 was applied to the heated golf ball bodies with the air-gun. The paint was dried in the oven heated at 40° C. to form the painted golf balls having the paint film with the thickness of 10 µm. The application of the paint was conducted immediately after (A) the aqueous polyol composition and (B) the aqueous polyisocyanate were mixed. The surface temperature of the golf ball bodies when applying the paint, the appearance of the resultant painted golf ball, the evenness and the adhesion of the formed paint film were evaluated and the results thereof were also shown in Tables 3 and 4.

TABLE 3

|                    |                                                       | Painted golf ball                                                                              |                               | 1     | 2     | 3     | 4     | 5     | 6     | 7     | 8     |
|--------------------|-------------------------------------------------------|------------------------------------------------------------------------------------------------|-------------------------------|-------|-------|-------|-------|-------|-------|-------|-------|
| Paint              | Formulation                                           | (A)                                                                                            | (a-1) Aqueous acrylic polyol  | 20    | 35    | 45    | 56    | 35    | 35    | 35    | 35    |
|                    |                                                       | Aqueous polyol composition                                                                     | (a-2) Aqueous urethane polyol | 30    | 15    | 5     | 24    | 15    | 15    | 15    | 15    |
|                    |                                                       |                                                                                                | (a-3) Aqueous urethane resin  | 50    | 50    | 50    | 20    | 50    | 50    | 50    | 50    |
|                    |                                                       | (B)                                                                                            | (b-1) HDI derivative          | 69    | 50.25 | 37.5  | 80.25 | 50.25 | 50.25 | 42    | 83.25 |
|                    |                                                       |                                                                                                | (b-2) IPDI derivative         | 23    | 16.75 | 12.5  | 26.75 | 16.75 | 16.75 | 14    | 27.75 |
|                    |                                                       | Non-volatile of (A) aqueous polyol composition (mass %)                                        |                               | 50.6  | 44.3  | 40.1  | 52.9  | 44.3  | 44.3  | 44.3  | 44.3  |
|                    |                                                       | Viscosity (mPa · s)                                                                            |                               | 130   | 155   | 160   | 165   | 155   | 155   | 145   | 175   |
|                    |                                                       | Mass ratio of (a-1)/(a-2) in (A) Aqueous polyol composition                                    |                               | 40/60 | 70/30 | 90/10 | 70/30 | 70/30 | 70/30 | 70/30 | 70/30 |
|                    |                                                       | Mass ratio of (b-1)/(b-2) in (B) Aqueous polyisocyanate                                        |                               | 75/25 | 75/25 | 75/25 | 75/25 | 75/25 | 75/25 | 75/25 | 75/25 |
|                    |                                                       | Molar ratio (NCO/OH) of NCO of (B) aqueous polyisocyanate/OH of (A) aqueous polyol composition |                               | 1.5   | 1.5   | 1.5   | 1.5   | 1.5   | 1.5   | 1.25  | 2.5   |
| Applying condition | Temp. (° C.) of preserving golf ball                  |                                                                                                |                               | 60    | 60    | 60    | 60    | 35    | 80    | 60    | 60    |
| Property           | Surface temp. (° C.) of golf ball when applying paint |                                                                                                |                               | 55    | 55    | 55    | 55    | 33    | 72    | 55    | 55    |
|                    | Appearance of golf ball                               |                                                                                                |                               | F     | G     | E     | G     | G     | G     | G     | G     |
|                    | Evenness of film thickness                            |                                                                                                |                               | G     | G     | G     | G     | G     | G     | G     | G     |
|                    | Adhesion of paint film                                |                                                                                                |                               | E     | G     | G     | F     | G     | G     | G     | G     |

TABLE 4

|                    |                                                       | Painted golf ball                                                                              |                               | 9     | 10    | 11    | 12    | 13    | 14    | 15    | 16    |
|--------------------|-------------------------------------------------------|------------------------------------------------------------------------------------------------|-------------------------------|-------|-------|-------|-------|-------|-------|-------|-------|
| Paint              | Formulation                                           | (A)                                                                                            | (a-1) Aqueous acrylic polyol  | 35    | 35    | 35    | 63    | 35    | 35    | 35    | 35    |
|                    |                                                       | Aqueous polyol composition                                                                     | (a-2) Aqueous urethane polyol | 15    | 15    | 15    | 27    | 15    | 15    | 15    | 15    |
|                    |                                                       |                                                                                                | (a-3) Aqueous urethane resin  | 50    | 50    | 50    | 10    | 50    | 50    | 50    | 50    |
|                    |                                                       | (B)                                                                                            | (b-1) HDI derivative          | 59.4  | 38    | 32    | 90    | 50.25 | 50.25 | 36.75 | 100.5 |
|                    |                                                       |                                                                                                | (b-2) IPDI derivative         | 0.6   | 38    | 48    | 30    | 16.75 | 16.75 | 12.25 | 33.5  |
|                    |                                                       | Non-volatile of (A) aqueous polyol composition (mass %)                                        |                               | 44.3  | 44.3  | 44.3  | 55.7  | 44.3  | 44.3  | 44.3  | 44.3  |
|                    |                                                       | Viscosity (mPa · s)                                                                            |                               | 155   | 155   | 155   | 170   | 155   | 155   | 140   | 180   |
|                    |                                                       | Mass ratio of (a-1)/(a-2) in (A) Aqueous polyol composition                                    |                               | 70/30 | 70/30 | 70/30 | 70/30 | 70/30 | 70/30 | 70/30 | 70/30 |
|                    |                                                       | Mass ratio of (b-1)/(b-2) in (B) Aqueous polyisocyanate                                        |                               | 99/1  | 50/50 | 40/60 | 75/25 | 75/25 | 75/25 | 75/25 | 75/25 |
|                    |                                                       | Molar ratio (NCO/OH) of NCO of (B) aqueous polyisocyanate/OH of (A) aqueous polyol composition |                               | 1.5   | 1.5   | 1.5   | 1.5   | 1.5   | 1.5   | 1.1   | 3     |
| Applying condition | Temp. (° C.) of preserving golf ball                  |                                                                                                |                               | 60    | 60    | 60    | 60    | R.T.  | 90    | 60    | 60    |
| Property           | Surface temp. (° C.) of golf ball when applying paint |                                                                                                |                               | 55    | 55    | 55    | 55    | R.T.  | 83    | 55    | 55    |
|                    | Appearance of golf ball                               |                                                                                                |                               | G     | G     | F     | G     | G     | P     | P     | P     |
|                    | Evenness of film thickness                            |                                                                                                |                               | G     | G     | G     | G     | P     | G     | G     | G     |
|                    | Adhesion of paint film                                |                                                                                                |                               | G     | G     | F     | P     | G     | G     | G     | P     |

R.T.: Room Temperature

Notes on Tables 3 and 4:

Formulation: mass parts (based on non-volatiles)

Aqueous acrylic polyol: an aqueous acrylic polyol (hydroxyl value: 108 mgKOH/g, average number of hydroxyl group: 28.8, glass transition temperature: 46°C., non-volatile: 46 mass %, weight average molecular weight: 15,000) available from SHINTO PAINT

Aqueous urethane polyol: "FLEXOREZ (registered trademark) UD-350W" (hydroxyl value: 325 mgKOH/g, average number of hydroxyl group: 2.3, non-volatile: 88 mass %, weight average molecular weight 400) available from King Industries, Inc.

Aqueous urethane resin: "SUPERFLEX (registered trademark) 300" (glass transition temperature: -40°C., Non-volatile content: 30 mass %, Elongation: 1500%) available from Dai-ichi Kogyo Seiyaku Co., Ltd

HDI derivative: "Bayhydur (registered trademark) 305" (NCO content: 16.2 mass %, non-solvent) available from Sumika Bayer Urethane Co., Ltd.

IPDI derivative: "Bayhydur (registered trademark) 401-70" (NCO content: 9.4 mass %, non-volatile: 70 mass %) available from Sumika Bayer Urethane Co., Ltd.

Painted golf balls No. 1 to 11 are the painted golf balls obtained by applying a two-component curing type urethane-based aqueous paint to a golf ball body having a surface temperature ranging from 30°C. to 80°C. These painted golf ball were excellent in gloss of the paint film, the evenness of the paint film, and the adhesion of the paint film to the surface of the golf ball body. Among them, the golf ball No. 11 is the case that the mixing ratio of (b-1) the hexamethylene diisocyanate derivative and (b-2) the isophorone diisocyanate derivative were mixed in a ratio of 40 mass %/60 mass % (total 100 mass %). The appearance of the painted golf ball and the adhesion of the paint film were slightly lowered.

The painted golf ball No. 12 is the case that the amount of (a-3) the aqueous urethane resin is low. The adhesion of the paint film was lowered. The painted golf ball No. 13 is the case that the two-component curing type urethane-based aqueous paint was applied to a golf ball body having a surface temperature of the room temperature (about 23°C.). In this case, the sagging of the applied paint was not sufficiently improved, and thus the evenness of the paint film was low. The painted golf ball No. 14 is the case that the two-component curing type urethane-based aqueous paint was applied to

a golf ball body having a surface temperature of 83°C. The appearance of the golf ball was low.

The painted golf ball No. 15 is the case that the molar ratio (NCO/OH) of the isocyanate group (NCO) of (B) the aqueous polyisocyanate to the hydroxyl group (OH) of (A) the aqueous polyol composition was 1.1. In this case, the leveling effect due to the isocyanate group was not obtained and thus the appearance of the painted golf ball was low.

The painted golf ball No. 16 is the case that the molar ratio (NCO/OH) of the isocyanate group (NCO) of (B) the aqueous polyisocyanate to the hydroxyl group (OH) of (A) the aqueous polyol composition was 3.0. In this case, since the isocyanate group was in excess, the obtained paint film was brittle, and the adhesion of the paint film was low. Further, the appearance of the painted golf ball was low, because the isocyanate group in excess reacted with water and carbon dioxide gas generated.

(5) Formation of Paint Film for Golf Balls No. 17 to No. 34

The surfaces of the obtained golf ball bodies were subjected to the sandblast treatment. Then, the two-component curing type aqueous urethane-based paint shown in Tables 5 and 6 was applied to the heated golf ball bodies with the air-gun. The paint was dried in the oven heated at 40°C. to form the painted golf balls having the paint film with the thickness of 10 µm. The application of the paint was conducted immediately after (A) the aqueous polyol composition and (B) the aqueous polyisocyanate were mixed.

The golf ball bodies were placed in the rotating member 1 shown in FIG. 1, which rotated at 3,000 rpm. The application of the paint film was conducted under the conditions shown in tables 5 and 6, by spacing a spray distance (7 cm) between the air gun and the golf ball body and moving the air gun in a up and down direction. Except golf balls No. 21 and No. 30, the painting interval in the overpainting operation was set to 1.0 second. In golf ball No. 21, the paint was first applied to the surface of the golf ball body, the applied paint was dried at 40°C. for 24 hours, and then the paint was applied second time. Application of the paint was conducted in the spraying conditions of spraying air pressure: 0.15 MPa, compressed air tank pressure: 0.10 MPa, and painting time per one time: 1 second, atmosphere temperature: 20°C. to 27°C., and atmosphere humidity: 65% or less.

The appearance of the resultant painted golf ball, the evenness and the adhesion of the formed paint film were evaluated and the results thereof were also shown in Tables 5 and 6.

TABLE 5

|                       |                                                                                                   | Painted golf ball                             |                                                                                                        | 17             | 18             | 19             | 20             | 21             | 22             | 23             | 24             | 25 |
|-----------------------|---------------------------------------------------------------------------------------------------|-----------------------------------------------|--------------------------------------------------------------------------------------------------------|----------------|----------------|----------------|----------------|----------------|----------------|----------------|----------------|----|
| Paint                 | Formulation                                                                                       | (A)<br>Aqueous<br>polyol<br>composition       | (a-1) Aqueous acrylic<br>polyol<br>(a-2) Aqueous urethane<br>polyol<br>(a-3) Aqueous urethane<br>resin | 20             | 35             | 45             | 56             | 35             | 35             | 35             | 35             | 35 |
|                       | (B)<br>Aqueous<br>polyisocyanate                                                                  | (b-1) HDI derivative<br>(b-2) IPDI derivative | 69<br>23                                                                                               | 50.25<br>16.75 | 37.5<br>12.5   | 80.25<br>26.75 | 50.25<br>16.75 | 50.25<br>16.75 | 42<br>14       | 83.25<br>27.75 | 59.4<br>0.6    |    |
|                       | Non-volatile of (A) aqueous polyol composition<br>(mass %)                                        |                                               | 50.6<br>50.6                                                                                           | 44.3<br>40.1   | 50<br>52.9     | 50<br>44.3     | 50<br>44.3     | 50<br>44.3     | 50<br>44.3     | 50<br>44.3     | 50<br>44.3     |    |
|                       | Mass ratio of (a-1)/(a-2) in (A) Aqueous polyol<br>composition                                    |                                               | 40/60<br>70/30                                                                                         | 90/10<br>70/30 | 70/30<br>70/30 | 70/30<br>70/30 | 70/30<br>70/30 | 70/30<br>70/30 | 70/30<br>70/30 | 70/30<br>70/30 | 70/30<br>70/30 |    |
|                       | Mass ratio of (b-1)/(b-2) in (B) Aqueous polyisocyanate                                           |                                               | 75/25<br>1.5                                                                                           | 75/25<br>1.5   | 75/25<br>1.5   | 75/25<br>1.5   | 75/25<br>1.5   | 75/25<br>1.5   | 75/25<br>1.25  | 75/25<br>2.5   | 99/1<br>1.5    |    |
|                       | Molar ratio (NCO/OH) of NCO of (B) aqueous<br>polyisocyanate/OH of (A) aqueous polyol composition |                                               |                                                                                                        |                |                |                |                |                |                |                |                |    |
|                       | Non-volatile (mass %)                                                                             |                                               | 27                                                                                                     | 32             | 35             | 37             | 32             | 32             | 33             | 40             | 32             |    |
|                       | Viscosity (mPa · s)                                                                               |                                               | 130<br>130                                                                                             | 155<br>160     | 160<br>165     | 165<br>155     | 155<br>155     | 155<br>145     | 145<br>175     | 175<br>155     |                |    |
| Applying<br>condition | Times of overpainting                                                                             |                                               | 2<br>2                                                                                                 | 2<br>2         | 2<br>2         | 2<br>2         | 2<br>3         | 2<br>2         | 2<br>2         | 2<br>2         |                |    |
|                       | Applied amount of Paint per one time (mg/per 1<br>golf ball)                                      |                                               | 40<br>40                                                                                               | 40<br>40       | 40<br>40       | 40<br>40       | 40<br>27       | 40<br>40       | 40<br>40       | 40<br>40       |                |    |

TABLE 5-continued

| Painted golf ball                   |                              | 17   | 18   | 19  | 20  | 21 | 22 | 23   | 24   | 25  |
|-------------------------------------|------------------------------|------|------|-----|-----|----|----|------|------|-----|
| Property of<br>Painted<br>Golf ball | Thickness of Paint film (μm) | 10.1 | 10.3 | 9.8 | 9.9 | 10 | 10 | 10.3 | 10.1 | 9.8 |
|                                     | Appearance of golf ball      | F    | G    | E   | G   | G  | G  | G    | G    | G   |
|                                     | Evenness of film thickness   | G    | G    | G   | G   | G  | G  | G    | G    | G   |
|                                     | Adhesion of paint film       | E    | G    | G   | F   | G  | G  | G    | G    | G   |

TABLE 6

| Painted golf ball                   |                                                                                                | 26                                                                                                                                 | 27             | 28             | 29             | 30             | 31             | 32             | 33             | 34             |                |
|-------------------------------------|------------------------------------------------------------------------------------------------|------------------------------------------------------------------------------------------------------------------------------------|----------------|----------------|----------------|----------------|----------------|----------------|----------------|----------------|----------------|
| Paint                               | Formulation                                                                                    | (A)<br>Aqueous polyol composition<br>(a-1) Aqueous acrylic polyol<br>(a-2) Aqueous urethane polyol<br>(a-3) Aqueous urethane resin | 35<br>15<br>50 | 35<br>15<br>50 | 35<br>15<br>10 | 63<br>15<br>50 | 35<br>15<br>50 | 35<br>15<br>50 | 35<br>15<br>50 | 35<br>15<br>50 | 20<br>30<br>50 |
|                                     | (B)<br>Aqueous polyisocyanate                                                                  | (b-1) HDI derivative<br>(b-2) IPDI derivative                                                                                      | 38<br>38       | 32<br>48       | 50.25<br>16.75 | 90<br>30       | 50.25<br>16.75 | 36.75<br>12.25 | 100.5<br>33.5  | 50.25<br>16.75 | 69<br>23       |
|                                     | Non-volatile of (A) aqueous polyol composition (mass %)                                        | 44.3<br>44.3                                                                                                                       | 44.3<br>55.7   | 44.3<br>44.3   | 44.3<br>44.3   | 44.3<br>44.3   | 44.3<br>44.3   | 44.3<br>44.3   | 44.3<br>44.3   | 50.6           |                |
|                                     | Mass ratio of (a-1)/(a-2) in (A) Aqueous polyol composition                                    | 70/30<br>70/30                                                                                                                     | 70/30<br>70/30 | 70/30<br>70/30 | 70/30<br>70/30 | 70/30<br>70/30 | 70/30<br>70/30 | 70/30<br>70/30 | 70/30<br>70/30 | 40/60          |                |
|                                     | Mass ratio of (b-1)/(b-2) in (B) Aqueous polyisocyanate                                        | 50/50<br>1.5                                                                                                                       | 40/60<br>1.5   | 75/25<br>1.5   | 75/25<br>1.5   | 75/25<br>1.5   | 75/25<br>1.1   | 75/25<br>3     | 75/25<br>1.5   | 75/25<br>1.5   |                |
|                                     | Molar ratio (NCO/OH) of NCO of (B) aqueous polyisocyanate/OH of (A) aqueous polyol composition |                                                                                                                                    |                |                |                |                |                |                |                |                |                |
|                                     | Non-volatile (mass %)                                                                          | 32<br>155                                                                                                                          | 32<br>155      | 32<br>155      | 40<br>170      | 32<br>155      | 30<br>140      | 42<br>180      | 10<br>155      | 70<br>250      |                |
|                                     | Viscosity (mPa · s)                                                                            |                                                                                                                                    |                |                |                |                |                |                |                |                |                |
| Applying condition                  | Times of overpainting                                                                          | 2<br>2                                                                                                                             | 4<br>2         | 2<br>1         | 1<br>2         | 2<br>2         | 2<br>2         | 2<br>2         | 2<br>2         | 2<br>2         |                |
| Property of<br>Painted<br>Golf ball | Applied amount of Paint per one time (mg/per 1 golf ball)                                      | 40<br>9.9                                                                                                                          | 40<br>10.1     | 40<br>20       | 40<br>10.1     | 80<br>10.5     | 40<br>10.2     | 40<br>9.7      | 40<br>9.8      | 40<br>9.9      |                |
|                                     | Thickness of Paint film (μm)                                                                   |                                                                                                                                    |                |                |                |                |                |                |                |                |                |
|                                     | Appearance of golf ball                                                                        | G<br>G                                                                                                                             | F<br>G         | G<br>G         | G<br>P         | P<br>G         | P<br>G         | P<br>G         | P<br>G         | P<br>G         |                |
|                                     | Evenness of film thickness                                                                     |                                                                                                                                    |                |                |                |                |                |                |                |                |                |
|                                     | Adhesion of paint film                                                                         | G<br>G                                                                                                                             | F<br>F         | G<br>G         | P<br>P         | G<br>G         | P<br>G         | P<br>G         | P<br>G         | P<br>G         |                |

## Notes on Tables 5 and 6

Formulation: mass parts (based on non-volatiles)

Details of the raw materials are shown in Notes on tables 3 and 4.

Painted golf balls No. 17 to 28 are the painted golf balls obtained by overpainting a two-component curing type urethane-based aqueous paint containing (A) an aqueous polyol composition and (B) an aqueous polyisocyanate to a golf ball body multiple times until a paint film has a desired thickness, such that an applied amount (dry mass) of the paint per one time ranges from 5 mg below 80 mg. These painted golf ball were excellent in gloss of the paint film, the evenness of the paint film, and the adhesion of the paint film to the surface of the golf ball body. Among them, the golf ball No. 27 is the case that the mixing ratio of (b-1) the hexamethylene diisocyanate derivative/(b-2) the isophorone diisocyanate derivative was 40 mass %/60 mass % (total: 100 mass %). The appearance of the painted golf ball and the adhesion of the paint film were slightly lowered.

The painted golf ball No. 29 is the case that the amount of (a-3) the aqueous urethane resin is low. The adhesion of the paint film was lowered. The painted golf ball No. 30 is the case that the two-component curing type urethane-based aqueous paint was applied to a golf ball body in an applied paint amount of 80 mg per one time. In this case, the sagging of the applied paint was not sufficiently improved, and thus the evenness of the paint film was low.

The painted golf ball No. 31 is the case that the mole ratio (NCO/OH) of the isocyanate group (NCO) of (B) the aqueous polyisocyanate to the hydroxyl group (OH) of (A) the aqueous polyol composition was 1.1. In this case, the leveling effect due to the isocyanate group was not obtained and thus the appearance of the painted golf ball was low.

The painted golf ball No. 32 is the case that the mole ratio (NCO/OH) of the isocyanate group (NCO) of (B) the aqueous polyisocyanate to the hydroxyl group (OH) of (A) the aque-

ous polyol composition was 3.0. In this case, since the isocyanate group was in excess, the obtained paint film was brittle, and the adhesion of the paint film was low. Further, the appearance of the painted golf ball was low, because the isocyanate group in excess reacted with water and carbon dioxide gas generated.

The painted golf ball No. 33 is the case that the non-volatile of the paint was less than 15 mass %. Since the applied paint amount (before dry) increased in order to obtain the desired film thickness, the applied paint sagged and thus the evenness of the paint film was low. The painted golf ball No. 34 is the case that the non-volatile of the paint was more than 60 mass %. Because of high viscosity of the paint, the leveling of the paint was lowered, and thus the appearance of the painted golf ball was low.

According to the present invention, it is possible to obtain the golf ball which is excellent in the gloss of the paint film, the even thickness of the paint film, and the adhesion of the paint film to the golf ball body. This application is based on Japanese Patent applications No. 2008-311112 filed on Dec. 5, 2008, No. 2008-321314 filed on Dec. 17, and No. 2009-257428 filed on Nov. 10, 2009, the contents of which are hereby incorporated by reference.

55 The invention claimed is:

1. A method for producing a golf ball comprising applying a two-component curing type urethane-based aqueous paint containing (A) an aqueous polyol composition and (B) an aqueous polyisocyanate to a golf ball body having a surface temperature ranging from 30° C. to 80° C., wherein,
  - (A) the aqueous polyol composition contains (a-1) an aqueous acrylic polyol, (a-2) an aqueous urethane polyol and (a-3) an aqueous urethane resin; a content of (a-3) the aqueous urethane resin in (A) the aqueous polyol composition ranges from 20 mass % to 80 mass %; and

a molar ratio (NCO/OH) of an isocyanate group of (B) the aqueous polyisocyanate to a hydroxyl group of (A) the aqueous polyol composition ranges from 1.25 to 2.50.

2. The method for producing the golf ball according to claim 1, wherein (a-3) the aqueous urethane resin has an elongation ranging from 100% to 2,000%.

3. The method for producing the golf ball according to claim 1, wherein (a-1) the aqueous acrylic polyol has a hydroxyl value ranging from 50 mgKOH/g to 150 mgKOH/g.

4. The method for producing the golf ball according to claim 1, wherein a blending ratio (a-1)/(a-2) (total: 100 mass %) of (a-1) the aqueous acrylic polyol to (a-2) the aqueous urethane polyol in (A) the aqueous polyol composition is 40 mass % to 90 mass % to 10 mass %.

5. The method for producing the golf ball according to claim 1, wherein (B) the aqueous polyisocyanate contains (b-1) hexamethylene diisocyanate and/or a derivative thereof, and (b-2) isophorone diisocyanate and/or a derivative thereof.

6. The method for producing the golf ball according to claim 5, wherein a blending ratio (b-1)/(b-2) (total: 100 mass %) of (b-1) hexamethylene diisocyanate and/or the derivative thereof to (b-2) isophorone diisocyanate and/or the derivative thereof is 50 mass % to 99 mass %/50 mass % to 1 mass %.

7. The method for producing the golf ball according to claim 1, wherein (a-1) the aqueous acrylic polyol has a hydroxyl value ranging from 50 mgKOH/g to 150 mgKOH/g; a blending ratio (a-1)/(a-2) (total: 100 mass %) of (a-1) the aqueous acrylic polyol to (a-2) the aqueous urethane polyol in (A) the aqueous polyol composition is 40 mass % to 90 mass %/60 mass % to 10 mass %; and (a-3) the aqueous urethane resin has an elongation ranging from 100% to 2,000%.

8. The method for producing the golf ball according to claim 7, wherein (B) the aqueous polyisocyanate contains (b-1) hexamethylene diisocyanate and/or a derivative thereof and (b-2) isophorone diisocyanate and/or a derivative thereof, in a blending ratio (b-1)/(b-2) (total: 100 mass %) of (b-1) hexamethylene diisocyanate and/or the derivative thereof to (b-2) isophorone diisocyanate and/or the derivative thereof being 50 mass % to 99 mass %/50 mass % to 1 mass %.

9. A painted golf ball produced by the method for producing the golf ball according to claim 1, comprising a golf ball body, and a paint film formed on the golf ball body.

10. A method for producing a golf ball comprising, overpainting a two-component curing type urethane-based aqueous paint containing (A) an aqueous polyol composition and (B) an aqueous polyisocyanate to a golf ball body multiple times until a paint film has a desired thickness, such that an applied amount (dry mass) of the paint per one time ranges from 5 mg below 80 mg, wherein,

(A) the aqueous polyol composition contains (a-1) an aqueous acrylic polyol, (a-2) an aqueous urethane polyol and (a-3) an aqueous urethane resin;

a content of (a-3) the aqueous urethane resin in (A) the aqueous polyol composition ranges from 20 mass % to 80 mass %;

a molar ratio (NCO/OH) of an isocyanate group of (B) the aqueous polyisocyanate to a hydroxyl group of (A) the aqueous polyol composition ranges from 1.25 to 2.50; and

a non-volatile content of the two-component curing type urethane-based aqueous paint ranges from 15 mass % to 60 mass %.

11. The method for producing the golf ball according to claim 10, wherein the desired thickness ranges from 4  $\mu\text{m}$  to 50  $\mu\text{m}$ .

12. The method for producing the golf ball according to claim 10, wherein a painting interval in the overpainting the two-component curing type urethane-based aqueous paint multiple times is longer than 0 second and 20 seconds or less.

13. The method for producing the golf ball according to claim 10, wherein the overpainting the two-component curing type urethane-based aqueous paint multiple times is conducted with an air gun under a spraying condition of a spraying air pressure: 0.01 MPa to 0.3 MPa, and an air pressure of a compressed air tank: 0.01 MPa to 0.3 MPa.

14. The method for producing the golf ball according to claim 10, wherein (a-3) the aqueous urethane resin has an elongation ranging from 100% to 2,000%.

15. The method for producing the golf ball according to claim 10, wherein (a-1) the aqueous acrylic polyol has a hydroxyl value ranging from 50 mgKOH/g to 150 mgKOH/g.

16. The method for producing the golf ball according to claim 10, wherein a blending ratio (a-1)/(a-2) (total: 100 mass %) of (a-1) the aqueous acrylic polyol to (a-2) the aqueous urethane polyol in (A) the aqueous polyol composition is 40 mass % to 90 mass %/60 mass % to 10 mass %.

17. The method for producing the golf ball according to claim 10, wherein (B) the aqueous polyisocyanate contains (b-1) hexamethylene diisocyanate and/or a derivative thereof, and (b-2) isophorone diisocyanate and/or a derivative thereof.

18. The method for producing the golf ball according to claim 17, wherein a blending ratio (b-1)/(b-2) (total: 100 mass %) of (b-1) hexamethylene diisocyanate and/or the derivative thereof to (b-2) isophorone diisocyanate and/or the derivative thereof is 50 mass % to 99 mass %/50 mass % to 1 mass %.

19. A painted golf ball produced by the method for producing the golf ball according to claim 10, comprising a golf ball body, and a paint film formed on the golf ball body.